

Aug. 12, 1941.

J. A. M. VAN LIEMPT

2,252,241

FLASH LAMP

Filed March 11, 1938



INVENTOR  
JOHANNES ANTONIUS MARIA VAN LIEMPT

BY

*De B. Sturman*  
ATTORNEY.

## UNITED STATES PATENT OFFICE

2,252,241

## FLASH LAMP

Johannes Antonius Maria van Liempt, Eindhoven, Netherlands, assignor, by mesne assignments, to Hartford National Bank and Trust Company, Hartford, Conn., as trustee

Application March 11, 1938, Serial No. 195,382  
In Germany March 30, 1937

6 Claims. (Cl. 52—24)

My invention relates to flash lamps, and more particularly to a flasher material for such lamps, i. e., a material which burns to emit the actinic light of the lamp.

For this purpose, it has been proposed to use aluminum or magnesium, the aluminum being preferably used in an extremely thin form, such as foil, and the magnesium being even suitable when the material is comparatively thick. However, magnesium has the disadvantage that it is very difficult to work, for instance rolled or drawn into a thin foil or a wire, whereas aluminum can readily be worked, more particularly rolled to thin sheets.

The main object of my invention is to produce a flash material that can be mechanically worked even more easily than aluminum, and can be more easily drawn into the form of a wire.

Another object is to produce a material which can be ignited more readily than aluminum and whose rate of combustion while emitting actinic light proceeds more rapidly than with aluminum itself.

A further object is to produce a material which develops per unit weight, a larger quantity of light than does pure aluminum or pure magnesium.

Further objects of the invention will appear as the description progresses.

In accordance with the invention I mix or alloy aluminum with either zinc or cadmium or a mixture thereof—which metals alone burn with hardly any actinic effect—and thereby obtain flasher materials which are superior to either pure aluminum or pure magnesium. More particularly I use as the flasher material a band, wire or foil consisting of an aluminum-zinc alloy containing not more than 20 per cent by weight of zinc, or a mixture of aluminum and cadmium containing not more than 80 per cent by weight of cadmium, or a mixture of aluminum, cadmium and zinc containing not more than 20 per cent by weight of zinc.

In order that my invention may be clearly understood and readily carried into effect I shall describe the same in more detail with reference to the accompanying drawing in which the single figure is a partly-sectionized side view of a flash lamp embodying the invention.

The flash lamp illustrated in the drawing comprises a container 1 of light-transmitting material such as glass having a press 2. Supported from press 2 by means of two supports 3 is an igniter or primer 4 such as a filament

provided with an explosive material, for instance a mixture of pulverized aluminum or zirconium and an oxidizing agent such as lead dioxide. Within the container is a flasher material 5 in the form of a clew of thin wire having a perimeter of the order of 300 microns or less. The lamp is filled with a gaseous filling such as oxygen or a gas containing oxygen.

In accordance with the invention the flasher material 5 consists of an aluminum-zinc alloy containing not more than 20% by weight of zinc, a mixture of aluminum and cadmium containing not more than 80% by weight of cadmium, or a mixture of aluminum, cadmium and zinc containing not more than 20% by weight of zinc.

Above I have referred to both alloys and mixtures, and to clarify this it should be noted that aluminum and cadmium alloy only partially in the literal meaning of the term. However, when there is more than 5% cadmium, the non-alloying cadmium particles can be sufficiently finely distributed throughout the molten aluminum-cadmium alloy by stirring vigorously, so that pseudo-alloys containing substantially more than 5% cadmium, for instance 60%, can be obtained. Such pseudo-alloys can be drawn into a wire as readily as the ordinary alloys. I have found that an aluminum-cadmium alloy containing not more than 5% cadmium burns more readily than does pure aluminum, and has a flash-time which, for the same thickness of wire, is not much shorter than that of aluminum itself. However, the above-mentioned pseudo-alloys have a much shorter flash-time with an equal quantity of emitted light, and this time is even shorter than that of aluminum and that of aluminum-zinc alloys containing not more than 20% by weight of zinc.

The invention may also be carried into effect when using aluminum-cadmium-zinc mixtures containing not more than 20% by weight of zinc and whose properties correspond to those of the alloys or mixtures referred to above.

I have found that the following specific alloys and mixtures give very good results: Aluminum-zinc containing 17% by weight of zinc, aluminum-cadmium containing 40% by weight of cadmium and aluminum-zinc-cadmium containing 6% by weight of zinc and 9% by weight of cadmium.

The flasher materials according to the invention have the advantage over pure aluminum that the flash time, i. e., the time required for the combustion, is considerably shorter. This

can be determined by observing the light-time curve of the aluminum and of the alloys or mixtures according to the invention. In addition I have found that the flash-time of the flasher materials of the present invention becomes shorter as the zinc content increases, and as the cadmium content increases to about 80%.

Furthermore, the flasher material of the invention can be readily drawn into a very thin wire, which is of great advantage. More particularly the flasher material is preferably used in the form of a thin wire or band, instead of a foil, because drawing the material into a thin wire or band is, from a mechanical viewpoint, much easier and cheaper than rolling it into thin foil.

Although aluminum-magnesium alloys containing more than 85% or less than 13% of magnesium are entirely satisfactory as flasher materials and can be readily drawn into thin wires, the flasher material according to the invention has the additional advantage over such alloys that when in the form of wire the quantity of light developed per unit length is about 10% greater.

The word "alloy" as used in the claims is to be understood to include both a true alloy as well as a pseudo-alloy or mixture.

While I have described my invention in connection with flash-lamps in which the flasher material is in the form of a wire, the material may be in other forms such as a foil or a band. Therefore I do not wish to be limited to the specific applications and examples described but

desire the appended claims to be construed as broadly as permissible in view of the prior art.

What I claim is:

- 5 1. In a photo-flash lamp, a flasher material consisting of an alloy of aluminium, zinc, and cadmium in the proportion of about 6% by weight of zinc, of about 9% by weight of cadmium, and the remainder aluminium.
- 10 2. In a photo-flash lamp, a flasher material consisting of an alloy of aluminium and zinc in the proportion of about 1% to 20% by weight of zinc and the remainder aluminium.
- 15 3. In a photo-flash lamp, a flasher material consisting of an alloy of aluminium and zinc in the proportion of about 17% by weight of zinc and the remainder aluminium.
- 20 4. In a photo-flash lamp, a flasher material consisting of an alloy of aluminium and cadmium in the proportion of about 1% to 80% by weight of cadmium and the remainder aluminium.
- 25 5. In a photo-flash lamp, a flasher material consisting of an alloy of aluminium and cadmium in the proportion of about 40% by weight of cadmium and the remainder aluminium.
- 30 6. In a photo-flash lamp, a flasher material consisting of an alloy of aluminum and at least one of the metals zinc and cadmium in the proportion of 99 to 20% by weight of aluminum, and 1 to 80% by weight of zinc and cadmium, the zinc content lying between 0 and 20% by weight.

JOHANNES ANTONIUS MARIA VAN LIEMPT.